

## UNITED STATES PATENT OFFICE

2,042,972

ELECTRICAL RESISTANCE ELEMENT AND  
ALLOY THEREFOR

James L. Thomas, Garrett Park, Md., assignor to  
the Government of the United States, as repre-  
sented by the Secretary of Commerce

No Drawing. Original application November 22,  
1934, Serial No. 754,310. Divided and this ap-  
plication November 18, 1935, Serial No. 50,378

3 Claims. (Cl. 201—76)

(Granted under the act of March 3, 1883, as  
amended April 30, 1928; 370 O. G. 757)

The invention described herein may be manufactured and used by or for the Government of the United States for governmental purposes only without the payment of any royalty thereon.

5 This invention relates to a new and improved electrical resistance element, and is a division of my application Serial No. 754,310, filed Nov. 22nd, 1934.

Generally, in electrical measuring apparatus, 10 coils of wire are utilized and difficulty has always been encountered in obtaining a wire whose resistance remains stable or substantially constant. It is known that resistance changes with age and also with ordinary changes in laboratory temperature. The change which takes place with age may be due to chemical action of the air upon the surface of the wire, or to changes in the crystal arrangement therein.

Further, besides the stability, resistance alloys 15 should have low temperature coefficients of resistance in order that they may be readily measured to a high precision.

To the best of my knowledge, no alloy has been developed which is entirely free from changes in 20 resistance with time or with temperature, but special alloys have been developed for which the changes in resistance with temperature and time are comparatively small. "Manganin", an alloy of copper, manganese and nickel is the alloy most 25 generally used for this purpose at present, but this alloy does not possess the desired qualities to a sufficiently high degree.

I have conducted experiments with an alloy 30 consisting mostly of gold with a small addition of chromium. Specifically, my research and tests have included a number of different alloys composed of gold with the addition of approximately from 1.5 to 5 percent of chromium by weight. As 35 a result of the tests I have found the most desirable mixture is approximately 2.1 percent of chromium and the remainder gold. Moreover, I have discovered that the addition of 1.5 to 5 percent of chromium to gold produces alloys having 40 very small temperature coefficients of electrical resistance and that the temperature coefficient of the alloys depends upon the proportions of the two ingredients.

The first difficulty encountered was to discover 45 a method by which the two ingredients could be

properly alloyed, and this method is described and claimed in my co-pending application, to which reference has been made above.

The following table is illustrative of the temperature-resistance changes of a 10-ohm coil of 5 the 2.1 percent chromium alloy baked at a temperature of 200° C. to bring its value to zero:

| Temperature | Resistance           |
|-------------|----------------------|
| 20° C.      | 9.99561 <sub>1</sub> |
| 22.5        | 9.99561 <sub>1</sub> |
| 25          | 9.99561 <sub>1</sub> |
| 27.5        | 9.99561 <sub>0</sub> |
| 30          | 9.99561 <sub>1</sub> |

The resistance of this coil was substantially independent of temperature throughout the entire interval 20–30° C. With manganin a minimum variation of about 10 parts per million would have been expected in this entire temperature interval, which is nearly a hundred times that of the 2.1 percent chromium alloy. In testing 10-ohm and 100-ohm coils the temperature resistance curves were found to be substantially identical in each case.

When manganin is used, in the construction 20 of resistance standards, the coils are usually kept for a year or more in order to reach a reasonably stable state, but with my alloy this ageing is not necessary, and, obviously, is greatly preferable to 30 the manganin.

As will be evident to those skilled in the art, my invention permits of changes in percentages of elements in the alloy without departing from the spirit thereof or the scope of the appended 35 claims.

What I claim is:

1. An electrical resistance element composed of an alloy comprised of gold and chromium, the chromium being in the percentage of from one to five percent and the gold constituting the remainder of the element.

2. An alloy comprising 2.1 percent of chromium and the remainder gold.

3. An alloy composed of gold and chromium, the chromium being in the percentage of from one to five percent and the gold constituting the remainder.

JAMES L. THOMAS.